

March 5, 1963

T. SENDZIMIR

3,079,975

PREVENTION OF COIL BREAKS

Filed July 2, 1956



INVENTOR.

TADEUSZ SENDZIMIR,

BY *Allen & Allen*

ATTORNEYS.

1

3,079,975

## PREVENTION OF COIL BREAKS

Tadeusz Sendzimir, Middletown, Ohio

(Armzen Co., Oxford Circle, Waterbury 12, Conn.)

Filed July 2, 1956, Ser. No. 595,224

9 Claims. (Cl. 153—54)

Some metals, such for example as low carbon steel after annealing, do not give uniformly over the whole stressed area when stressed beyond their yield point, but yield first along spaced, irregular lines roughly perpendicular to the direction of the stress. This may produce a defective surface appearance. The same phenomenon, when an attempt is made to bend a metal sheet, may produce a sharp break in direction rather than a smooth conformation to the desired shape. Thus it may be found impossible to form the material into a smooth cylinder, because sharp bends occurring therein tend to give it a multi-lateral configuration. Metals having such defects are generally said to be subject to "coil breaks" as a matter of convenient terminology.

This objectionable behavior of the metal is manifest, for example, in processes for continuously coating cold rolled low carbon steel strip with molten coating metal, which processes involve high temperature annealing. As examples of such procedures reference is made to United States Patents 2,110,893, 2,136,957, and 2,197,622 in the name of Tadeusz Sendzimir. After coating the strip is rapidly cooled and finally coiled or cut up into sheets which may be subject to coil breaks as set forth.

To eliminate this defect a flexing machine such as a roller leveler has been employed on the coated metal. Providing the gauge of the treated strip is not too light, the use of a roller leveler may be effective in the production of commercially acceptable products. As is well known, the leveler produces coil breaks but at such close intervals that the individual breaks cannot be detected by the eye, or will at least be so close together as not to interfere with the subsequent use of the product. In general, a leveler which can be depended upon to produce coil breaks separated by not more than three to four times the thickness of the strip will be found satisfactory.

However, for light gauges such as 0.015 inch and below known roller levelers are not capable of producing coil breaks close enough to one another in the product to make it commercially acceptable. Tension applied to the strip during leveling improves the operation of the device and yet the above named gauge is about the lower limit of permissible operation.

It is a primary object of the invention to provide a method and apparatus for flexing an annealed strip which may be depended upon to alleviate the difficulty above discussed even where the strip is of very light gauge.

It is an object of the invention to provide a method and apparatus which, while not limited for use on light gauge strip, will produce a strip which may be bent, formed or subjected to drawing operations without the formation of coil breaks or that appearance which is frequently termed "stretcher strains."

These and other objects of the invention which will be set forth hereinafter or will be apparent to one skilled in the art upon reading these specifications are accomplished by that construction and arrangement of parts and in that procedure of which an exemplary embodiment will now be described. Reference is made to the accompanying drawings wherein:

FIGURE 1 is a side elevation of the exemplary apparatus.

FIGURE 2 is a partial elevation on an enlarged scale of a portion of the apparatus shown in FIGURE 1.

FIGURE 3 is a partial end elevation taken from the right in FIGURE 1.

2

FIGURE 4 is a partial sectional view taken along the section line 4—4 of FIGURE 3.

FIGURE 5 is a partial sectional view taken along the section line 5—5 of FIGURE 4.

FIGURE 6 is a partial sectional view taken along the section line 6—6 of FIGURE 4.

In the practice of the invention the strip is passed between a small diameter roll properly supported to prevent deflection (or several such rolls) and an elastic medium exerting substantially uniform pressure on the strip parallel to the axis of the roll, the pressure being of sufficient magnitude to bend the strip continuously so as to make it conform to enough of the circumference of the small diameter roll to produce the desired effect.

15 The action is that of producing coil breaks so close to one another as to be indistinguishable, the distance between coil breaks being preferably of the order of 0.010 inch to 0.005 inch. Since the apparatus is designed to handle light gauge strip as well as heavier materials, the 20 rolls should be of quite small diameter, say  $\frac{1}{4}$  inch to one inch. These diameters are not necessarily limiting, and it is possible to vary the diameter of the rolls in accordance with the gauge of the strip, especially where the apparatus is to operate upon a relatively narrow range of 25 gauges. The elastic medium referred to above may be a rubber clad drum or roll of a diameter relatively large in relation to the other rolls.

By way of further preliminary explanation it has been found that in order to facilitate the aligning of the roll in 30 virtual parallelism with the axis of the elastic covered drum, it is preferable to provide an apparatus with two parallel flexing rolls. This results in a geometric arrangement which enables the drum to rest with respect to the rolls, thus making the apparatus self aligning to a certain extent. The strip undergoes the same flexing treatment 35 twice, which is beneficial.

It is also beneficial to tension the strip during treatment; and the greater the tension the less need be the pressure exerted by the elastic element to produce the 40 same results.

Yet another aspect of the invention has to do with introducing fluctuations in the pressure of the elastic medium against the rolls. The frequency of these fluctuations can be gauged to the desired distance between the 45 coil breaks produced by the apparatus. It has been found that the exertion of fluctuating pressure facilitates an exceedingly close spacing of the coil breaks because it obviates skips where the strip is sporadically subjected to a bending moment under a stress which is not strong 50 enough to produce the required strain. Under conditions of constant pressure the bending moment increases as the strip advances so that the coil breaks may be produced not at a predetermined distance but at some accidental distance coinciding with a point of least resistance in the 55 metal strip. A regular rhythmic surge in the pressure exerted by the elastic medium will cause the bends to take place regularly even under the most difficult conditions.

Referring to the various figures, the apparatus comprises spaced channel or beam members 1 and 2 which 60 bear journal bearings 3 and 7 for the shaft extensions of a drum 8 which bears on its surface a coating of elastic material 9. The drum 8 may be solid or hollow as desired, but in any event will have sufficient stiffness and will be mounted on shafts and in bearings of suitable size 65 to permit the exertion of the desired deflecting pressure. In FIGURE 1 the drum turns clockwise, and the strip 10 passes approximately 180° about its periphery. This is not a necessary limitation, since it is only necessary that the strip contact the drum in the area of operation of 70 flexing rolls indicated at 11 and 12. The strip may be tensioned in any way desired as by the use of pinch roll combinations or other pulling as retarding devices (not

shown) located ahead of and behind the treatment apparatus herein described.

Uprights 13 and 14 are provided at an end of each of the channels 1 and 2. Lever arms 15 and 16 are provided at one end to brackets 17 and 18. The other ends of the lever arms are connected by linkages to the pistons of fluid pressure cylinders mounted respectively on the channels 1 and 2. One of these cylinders is shown at 19 in FIGURE 1 the linkage being indicated at 20.

The lever arms are interconnected at about their center portions by a transverse beam 21 of substantial depth and stiffness. The lever arms may be unitary, or each may be made up of two parts interconnected by the beam. The beam may support on its top surface a motor and speed reducer for driving the flexing rolls together with vibrating means where employed. On its bottom surface it bears a flexing roll assembly in which the flexing rolls are supported throughout their working length.

At each end of the assembly there are plates 22 and 23. The deflecting rolls 11 and 12 are journaled at their ends in these plates. The plates are fastened to the underside of the beam 21 as by means of bolts or eyebolts 24 and 25. Provision may usefully be made for lateral adjustment of the plates 22 and 23. This may be accomplished by means of bolts 26 and 27, the bolts being provided with lock nuts and threaded into ears 28 and 29 on the beam. The bolts 24 and 25 may engage in slots in the webs of the beam.

Between the end plates 22 and 23 there is a series of spaced, plate-like supports 30 resting against the beams. The series may be threaded on shaft-like members 31 and 32 with the individual plates of the series held in spaced relationship by collars 33 surrounding the shafts. At their ends the shafts 31 and 32 may be threaded and provided with nuts 34 and 35 (FIGURE 5). The plates 30 serve as thrust supports for shafts 36, 37 and 38, on which are journaled series of casters 39, 40 and 41. The casters are spaced along the shafts so as to lie between the plates 30; and the deflecting rolls 11 and 12 are engaged by the casters as best shown in FIGURE 4 so as to be supported throughout their working lengths as will be evident. Any tendency of the thin rolls 11 and 12 to deflect is taken up by the casters and transferred to the beam 21 by the plates 30. The ends of the shafts 36, 37 and 38 may be mounted in the end plates 22 and 23. It is not necessary that they be journaled therein if the casters are mounted rotatably on the shafts. The casters may take several forms; but preferably they are short rollers mounted by means of ball or roller bearings on the shafts. The shafts 36, 37 and 38 may have center perforations as shown through which lubricant can be fed to the casters.

It is preferred to drive the flexing rolls 11 and 12. To this end they may be provided with sprockets 42 and 43 connected by means of a chain 44 to the sprocket 45 of a speed reducer 46. The speed reducer will be driven by a suitable electric motor (not shown) but also mounted on the beam 21. It is preferred to drive the rolls through a slip clutch or overrunning clutch (47 in FIGURE 3) which will keep the rolls turning at a minimum speed while leaving them free to attempt a faster speed should conditions require. A tightener for the chain 44 may be provided as at 48.

When fluid pressure is applied to the cylinders 19, a corresponding force multiplied by the leverage of the lever arms 15 and 16, will be applied to the flexing rolls 11 and 12 to force them into the elastic covering 9 of the drum 8. Strip 10 is flexed by the rolls 11 and 12 as most clearly shown in FIGURE 4, thereby producing the necessary tempering effect to avoid subsequent coil breaks.

By the means indicated a strip subject to coil breaks may be successfully treated for the elimination of this defect even though of very light gauge. Where the strip has been coated with molten metal or has been annealed,

the flexing operation should take place just prior to the coiling or shearing of the strip, i.e. at the point in the line where the strip temperature is lowest. It has been found that if the temperature of the metal during the mechanical working herein taught is too high, the physical properties of the strip and especially its elongation may suffer. It is also possible with some materials that the phenomenon of "ageing" may proceed at too rapid a rate.

In instances where (as shown) the strip 10 follows the periphery of the drum 8 for a substantial distance provision may be required for insuring proper tracking of the strip, especially where the strip has or may have a camber, as often happens with material rolled on 4-hi mills. The drum 8 may be given a degree of crown, or its axis may be made adjustable in the bearings 3 and 7. Means for the adjustment of the flexing roll combination has been described above. In the specific embodiment of the apparatus, a convenient way of insuring tracking lies in varying the pressures exerted by the lever arms 15 and 16. This can be readily accomplished by varying the fluid pressures in the cylinders 19. It will be obvious that the pressure at the low pressure side should always be enough to flex-temper the strip; but within this limitation the tracking can be readily controlled by differential variation of the pressures. The tracking is controlled by pressing the strip more or less into the elastic medium at one side of the strip as compared with the other. The tracking may be made automatic by connecting any known strip position indicator through suitable servo-mechanisms to pressure control means for the cylinders. A typical strip position indicator is a light roller contacting the edge of the strip under light spring pressure.

The value of the use of vibration or deliberately produced fluctuations of pressure has already been indicated. Such variations in pressure may conveniently be attained by attaching to the beam 21 a suitable vibrator (not shown). The vibrator may be any suitable mechanical, pneumatic, magnetic or electric device. Satisfactory results have also been attained by using flexing rolls having a degree of "chatter" such as may be involuntarily obtained in grinding such rolls. In attempting to produce chatter the rolls may be fluted in grinding with a minute pitch, or a similar treatment could be applied to the surfaces of the casters.

Rolls which are characterized by chatter and are fluted so as to have a polygonal section have a higher coefficient of friction while in contact with the strip than smooth rolls. Under these circumstances the drive for the flexing rolls may be omitted. The drive is usually provided as a safety measure to prevent the small flexing rolls skidding on the surface of the strip. Rolls which are rough, and especially fluted rolls, have sufficient coefficient of friction to be safe in this regard. As indicated above the drive need not be precisely timed, and preferably includes an overrunning clutch 47, enabling the rolls to adopt a higher speed as determined by the strip. Yet if the drive by contact with the strip should fail because the strip is too slippery, the chain drive takes over until drive by the strip is re-established.

Instances may be encountered in which a uniform degree of deflection is not desirable across the entire width of the strip. For example, in galvanized strip there may be a heavier deposit of zinc at the edges. Thus that degree of deflection which is desirable in the midsection of the strip may produce over-rolling at the edges which, if permitted to continue, would interfere with the guiding of the strip or the desired qualities of the final product.

As set forth above, the surface of the elastic medium on the drum may be contoured or the small rolls may be tapered near their ends or otherwise profiled to the most desirable shape. It is also possible to configure the casters in such a way that a controlled deflection of the small rolls will occur, or the bearings of the casters may be arranged (adjustably or not) to permit a controlled de-

flexion. Any or all of these expedients may be employed.

Modifications may be made in the invention without departing from the spirit of it. The effect desired can be obtained through the use of a single flexing roller operating against an elastic medium. For reasons given above two parallel rollers are preferred. But additional rollers may be employed if desired. The invention having been described in an exemplary embodiment, what is claimed as new and desired to be secured by Letters Patent is:

1. A process of treating light gauge metallic strip of substantial width to produce a strip that is virtually free from coil breaks in subsequent treatment, which process comprises passing a strip having a gauge not substantially greater than 0.015 in. between an elastic medium on one side and a small diameter roll on the other, the diameter of said roll being substantially .25 to 1.0 in. and chosen in accordance with the gauge of the strip to control the spacing of the breaks formed therein, said roll having a length at least equal to the width of the strip being treated, exerting pressure between the said roll and the elastic medium such as to cause the strip to compress the elastic medium and thereby be caused to conform for a limited arc to the periphery of the small roll, and supporting the small roll throughout its working length to minimize deflection thereof in all directions, whereby to produce in said strip a continuous succession of coil breaks lying close together and substantially parallel to each other, including the step of varying the said pressure periodically at a frequency related to the travel of the strip such as to produce breaks of a desired separation.

2. The process claimed in claim 1 in which the fluctuation of pressure is accomplished by vibrating means acting through the said small diameter roll.

3. The process claimed in claim 1 in which the fluctuation of pressure is accomplished in part at least by the provision of a non-circular roll surface.

4. A process of flex-tempering metal strip which comprises passing the said strip over the surface of a rotating drum covered with an elastic medium and pressing the said strip into the said elastic medium from its side opposite the elastic medium by means of at least one small diameter roll while maintaining said roll against flexing throughout its effective working length, and controlling the tracking of said strip while being so treated, by differentially controlling the said pressure at opposite ends of the effective working length of said roll.

5. In apparatus for the purpose described, an elastic-covered rotary drum of relatively large diameter, and having a width sufficient to accommodate wide, thin-gauge metallic strip, at least two flexing rolls each having a diameter of substantially 0.25 to 1.0 inch and a length at least equal to the width of said rotary drum, said flexing rolls being axially disposed with respect to said drum, means for supporting said flexing rolls throughout their working length to minimize deflection in all directions, said means comprising a beam extending axially of said drum and mounting sets of casters contacting each of said flexing rolls, means urging said flexing rolls against said drum under sufficient pressure so that, when a metallic strip is interposed between said flexing rolls and said drum, said strip will be caused to compress said elastic to cause said strip to conform to limited arcs of the peripheries of said flexing rolls, whereby coil breaks will be formed in said strip lying uniformly close together, and vibrating means attached to said beam.

6. In apparatus for the purpose described, an elastic-covered rotary drum of relatively large diameter, having a width sufficient to accommodate wide, thin-gauge metallic strip, at least two spaced flexing rolls each having a diameter of substantially 0.25 to 1.0 inch and a length at least equal to the width of said rotary drum, said flexing

rolls being axially disposed with respect to said drum, means supporting said flexing rolls throughout their working length to minimize deflection in all directions, said means including a beam extending axially of said drum and mounting sets of casters contacting said flexing rolls, means urging said flexing rolls against said drum under sufficient pressure so that, when a metallic strip is interposed between said flexing roll and said drum, said strip will be caused to compress said elastic to cause said strip to conform to limited arcs of the peripheries of said flexing rolls, whereby coil breaks will be formed in said strip lying uniformly close together, at least one rotating element other than said drum being of non-circular cross section productive of chatter.

10 7. In apparatus for the purpose described, an elastic-covered rotary drum of relatively large diameter, having a width sufficient to accommodate wide, thin-gauge metallic strip, at least two spaced flexing rolls each having a diameter of substantially 0.25 to 1.0 inch and a length at least equal to the width of said rotary drum, said flexing rolls being axially disposed with respect to said drum, means supporting said flexing rolls throughout their working length to minimize deflection in all directions, said means including a beam extending axially of said drum and mounting sets of casters contacting said flexing rolls, means for driving said flexing rolls, and means urging said flexing rolls against said drum under sufficient pressure so that, when a metallic strip is interposed between said flexing rolls and said drum, said strip will be caused to compress said elastic to cause said strip to conform to limited arcs of the peripheries of said flexing rolls, whereby coil breaks will be formed in said strip lying uniformly close together.

20 8. The structure claimed in claim 7 including means for adjustably positioning the said flexing rolls to align them with respect to the axis of said drum.

25 9. In apparatus for the purpose described, an elastic-covered rotary drum of relatively large diameter, having a width sufficient to accommodate wide, thin-gauge metallic strip, at least one flexing roll of relatively small diameter and of a length at least equal to the width of said rotary drum, said flexing roll being axially disposed with respect to said drum, means supporting said flexing roll throughout its working length to minimize deflection in all directions, said means including a beam extending axially of said drum and sets of casters thereon contacting said flexing roll, and means for urging said flexing roll toward said drum under pressure, said apparatus having a base in which said drum is journaled, said urging means comprising a pair of spaced levers, one at each end of said beam, said levers being mounted at one end pivotally on said base, said beam being mounted at its ends on central portions of said levers and each lever having a separately actuatable tensioning means connecting its other end with said base, whereby the pressure exerted by said flexing roll may be differentially controlled at the opposite ends of the effective working length of said roll to control the tracking of metallic strip passing through said apparatus.

References Cited in the file of this patent

UNITED STATES PATENTS

|           |            |               |
|-----------|------------|---------------|
| 175,365   | Marshall   | Mar. 28, 1876 |
| 447,295   | Brenner    | Mar. 3, 1891  |
| 1,032,907 | Hyde       | July 16, 1912 |
| 1,854,021 | Derby      | Apr. 12, 1932 |
| 1,930,562 | Krueger    | Oct. 17, 1933 |
| 2,059,993 | Hanson     | Nov. 3, 1936  |
| 2,060,400 | Nieman     | Nov. 10, 1936 |
| 2,176,872 | Hennessy   | Oct. 24, 1939 |
| 2,273,122 | Maussnest  | Feb. 17, 1942 |
| 2,486,844 | Hercik     | Nov. 1, 1949  |
| 2,612,934 | Dubosclard | Oct. 7, 1952  |